

# UNITED STATES PATENT OFFICE.

JOHN HENRY MACKLE, OF WATERVLIET, NEW YORK.

## LUBRICATING OIL OR GREASE.

1,191,328.

Specification of Letters Patent. Patented July 18, 1916.

No Drawing.

Application filed October 17, 1914. Serial No. 867,090.

To all whom it may concern:

Be it known that I, JOHN H. MACKLE, a citizen of the United States, and resident of the town of Watervliet, county of Albany, 5 State of New York, have invented certain new and useful Improvements in Lubricating Oils or Greases, of which the following is a specification.

Since the introduction of hydrocarbon 10 and other high speed and high temperature engines there has been a desire to obtain a suitable lubricating agent. The requirements are however of such a rigid character that when submitted to the test even the best 15 lubricants have been found wanting. The principal causes of failure are that lubricating oils will not withstand the required heat without becoming themselves affected with the heat to such an extent that they 20 smoke, burn and carbonize and therefore even though their presence is quite necessary it is also quite objectionable.

My invention consists of an oil that has been found satisfactory even after the most 25 rigid test, and one that although providing an entirely satisfactory lubrication does so without introducing into the cylinder of the engine readily deposited carbons that are later to be discharged as smoke, or retained 30 and deposited on the valves, the piston and the interior of the cylinder.

My invention consists of blending certain oils, that are high in lubricating qualities but low in carbon and treating the oils so 35 as to remove any impurities that might be contained therein.

In the best working of my invention I have selected cotton-seed oil and castor oil mixing them in about the following proportions: cotton-seed oil 85%, castor oil 15%. 40 I place the oils together in an open receptacle preferably of copper. I then heat the receptacle and continue it subject to the heat until the mixture ceases to foam or boil. I 45 then allow it to partially cool while sedimentation takes place, and after the impure matter has been boiled off or deposited within the receptacle by reason of this pre-

oxidization I draw off the pure oil, cool it to a proper temperature and it is ready for 50 use. I have found that in submitting the mixtures of oils to heat I can obtain any desirable degree of siccativeness but I have also found to obtain a heavy or light oil it is better to increase or decrease the percentage of castor oil for although an increase of the castor oil will not change the lubricating value of the resultant mixture, it will produce a heavier oil more suited to be used as a cylinder oil or for any other 55 purpose where a very heavy oil is found desirable.

My oil has many peculiar characteristics and I will briefly mention a few of the most important. I have already set forth that 60 the oil does not burn. Not only does it not burn but I have found that it will stand a very severe heat, the flash test being greater than that of either of the oils taken independently. 70

I believe that it would be quite possible to produce an oil having some of the characteristics of my oil by merely mixing certain proportions of castor oil and cotton-seed oil without heating and with only ordinary 75 sedimentation or filtration. Such an oil would, however, be of an inferior quality and would not contain some of the most important characteristics of my more perfect compound. 80

Having carefully and fully described my invention what I claim and desire to secure by Letters Patent is:

A lubricating oil which consists of cotton-seed oil 85% and castor oil 15% which mixture has been heated to boil off or deposit the impure matter or sediment and decanted for use as herein specified. 85

Signed at New York city, in the county of New York and State of New York this 6th 90 day of October 1914.

JOHN HENRY MACKLE.

Witnesses:

ALFRED T. GORMAN,  
ARTHUR PHELPS MARR.